

Patented Sept. 26, 1933

## UNITED STATES PATENT OFFICE

1,928,053

## DIE CAST ZINC BASE ALLOY PRODUCT

John R. Freeman, Jr., Waterbury, Conn., assignor to The American Brass Company, Waterbury, Conn., a corporation of Connecticut

No Drawing. Application December 17, 1931  
Serial No. 581,774

4 Claims. (Cl. 75-1)

This invention relates to die cast zinc base alloy products and has for its object the provision as a new article of manufacture of improved zinc base alloy products of this nature.

- 5 The design of the usual type of die casting machine is such that the mechanism is to a great extent completely immersed in the molten alloy to be cast. The mechanical requirements of the die casting process as carried out in the plunger or 10 goose-neck machines are such that many of the working parts of the machine must be constructed of iron or steel. These metals are subject to attack by molten zinc and zinc alloys and it is known from experience that to minimize this 15 attack sufficiently in order to obtain reasonable life from the machines it is necessary that at least 0.25% of aluminum be present in the alloys. It is known further that aluminum when present in zinc base alloys even in amounts less than 0.25% 20 causes a disintegration or intercrystalline corrosion to occur more especially in warm and humid atmospheres, but amounts less than 0.05 percent of aluminum may not be objectionable although it is preferred that the alloy be free 25 from aluminum, or at least contain not more than 0.05 percent. Magnesium also when present in zinc base alloys may under certain conditions, more particularly when the alloy is free or substantially free from aluminum, cause a similar 30 disintegration or intercrystalline corrosion to occur. Zinc base alloys containing aluminum are also subject to change in strength, more particularly in impact strength, with time even in the absence of moisture.
- 35 Improved zinc base alloys containing aluminum have been developed in which the degree of disintegration or intercrystalline oxidation has been reduced by the addition of elements other than aluminum such as copper and more particularly 40 magnesium. A committee on die cast metals and alloys of The American Society for Testing Materials has recently conducted an extensive series of tests to determine the most suitable alloy or alloys for adoption as standard alloys for 45 the industry. All of the alloys tested contained aluminum and of all the alloys tested only one alloy was found to be sufficiently stable, that is, free from disintegration or change in physical properties with time. This zinc base alloy has 50 the nominal composition of 4% aluminum, 3% copper and 0.05% magnesium, and the further requirement that the lead content shall be not greater than 0.01% and the cadmium and tin contents not greater than 0.005% respectively.
- 55 It is specified also that the zinc used for the

preparation of the alloy shall contain not more than 0.02% total impurities. The investigations of the above committee have shown that the use of very pure zinc is essential because of the deleterious effect of the impurities normally present in zinc, more particularly lead. It is known also that magnesium is essential in zinc alloys containing aluminum, even when very pure zinc is used to inhibit disintegration in humid atmospheres.

I have found that die cast zinc base alloy products made of an alloy of zinc and nickel and substantially free from aluminum and magnesium, more particularly an alloy containing from about 0.10 to about 10% of nickel and preferably 60 free from aluminum and magnesium, or containing less than 0.05% of aluminum and less than 0.05 percent magnesium may be prepared successfully and economically in a die casting machine in which the melting chamber is entirely separated from the casting mechanism. I have found that die cast zinc base alloy products containing the above noted proportions of nickel when free or substantially free from aluminum and magnesium are stable, that is, they do not 70 change in physical properties with time even when subjected to hot humid atmospheres for long period of time. The above range of nickel produces useful alloys, but the preferred range is from about 0.50% to about 1.5% of nickel.

75 For example there are given in the following tables the results of tests of a die cast zinc base alloy product prepared from a zinc nickel alloy substantially free from aluminum and magnesium, and of a similar die cast product of an alloy of zinc, copper, aluminum and magnesium. In the table the properties given for product designated (A) are typical for the new die cast products free or substantially free from 80 aluminum and magnesium for which Letters Patent are desired. The properties for product (B) are typical for die cast product containing 85 aluminum at present widely used in the industry.

100

## Composition of products

| Product | Zinc metal containing impurities less than | Nickel, percent | Copper, percent | Aluminum, percent | Magnesium, percent | 105 |
|---------|--------------------------------------------|-----------------|-----------------|-------------------|--------------------|-----|
| A       | 0.02                                       | 1.92            | 2.96            | Less than 0.01    | Less than 0.01     | 110 |
| B       | 0.02                                       |                 |                 | 4.24              | 0.07               |     |

## Physical properties as cast

| Product | Tensile strength, lbs./sq. in. | Elongation, percent in 2 inches | Impact resistance, ft. lbs. |
|---------|--------------------------------|---------------------------------|-----------------------------|
| 5       |                                |                                 |                             |
| A       | 21,600                         | 1.0                             | 2.53                        |
| B       | 42,154                         | 2.97                            | 11.83                       |

## 10 Physical properties after exposure to water vapor for 10 days at a temperature of 95° C.

| Product | Tensile strength, lbs./sq. in. | Elongation, percent in 2 inches | Impact resistance, ft. lbs. | Expansion of length of 6 inches, inches |
|---------|--------------------------------|---------------------------------|-----------------------------|-----------------------------------------|
| 15      |                                |                                 |                             |                                         |
| A       | 23,530                         | 1.5                             | 2.42                        | -0.0010                                 |
| B       | 37,650                         | 0.8                             | 1.26                        | +0.0107                                 |

- 20 It is evident that the new product is superior, its physical properties remaining practically constant under the extreme conditions of ten days exposure to water vapor at 95° C. whereas the product containing aluminum and magnesium shows considerable expansion and loss in impact resistance and elongation under the same conditions of exposure to heat and humidity.
- 25 It is apparent that the new product has a very greatly increased utility more particularly for use where permanence in dimensions or resistance to shock is required and where it would be subject to hot humid atmospheres.

In the preparation of the new zinc base alloy product I prefer to use zinc of highest purity as is required for alloys containing aluminum, but this is not essential although it is of considerable advantage and I mean to include as a part of this patent zinc base alloy products of composition stated prepared from zinc of high as well as commercial purity.

Having thus set forth the nature of my invention, what I claim is:

1. As a new article of manufacture a die cast product made of a zinc base alloy consisting of from about 0.10 percent to about 10 percent nickel and the balance zinc.
2. As a new article of manufacture a die cast product made of a zinc base alloy consisting of from about 0.50 percent to about 1.50 percent nickel and the balance zinc.
3. As a new article of manufacture a die cast product made of a zinc base alloy consisting of from about 0.10 percent to about 10 percent nickel and the balance high purity zinc metal containing not more than 0.02 percent total impurities.
4. As a new article of manufacture a die cast product made of a zinc base alloy consisting of from about 0.50 percent to about 1.50 percent nickel and the balance high purity zinc metal containing not more than 0.02 percent total impurities.

JOHN R. FREEMAN, JR. 105

35

110

40

115

45

120

50

125

55

130

60

135

65

140

70

145

75

150